

## UNITED STATES PATENT OFFICE

2,278,726

## MAGNESIUM BASE ALLOY

John C. McDonald, Midland, Mich., assignor to  
 The Dow Chemical Company, Midland, Mich.,  
 a corporation of Michigan

No Drawing. Application October 4, 1940,  
 Serial No. 359,681

3 Claims. (Cl. 75—168)

The invention relates to a magnesium base alloy. It more particularly concerns an alloy of this nature having improved physical properties such as high yield and tensile strengths.

Commercially pure magnesium has been used only to a limited extent as a structural material because of its relatively low tensile and yield strengths, although its light weight is oftentimes a highly desirable characteristic in making castings, forgings, extruded forms, and the like.

It is, therefore, the principal object of the invention to provide an alloy of magnesium which utilizes the light weight characteristic of magnesium and at the same time possesses superior strength characteristics.

Other objects and advantages will be apparent as the description of the invention proceeds.

My invention resides in the discovery that a magnesium base alloy composed of from 0.1 to 10 per cent of germanium, the balance being substantially all magnesium possesses the aforementioned properties. The term "magnesium" used herein and in the appended claims is intended to include magnesium containing the ordinary impurities that are found in the commercially pure metal, such as traces of iron, copper, nickel, and silicon. While the properties of high tensile and yield strengths are manifest over the entire range of composition indicated, the most desirable combination of properties is found in those alloys containing from 0.5 to 5 per cent of germanium.

A preferred composition having superior yield strength as well as highly improved tensile strength is one containing 0.8 per cent of germanium.

The following table which lists some of the properties of rolled sheet metal made from my new binary alloy and compares these properties with those of magnesium illustrates the improvement in yield strength and tensile strength of my new alloy over that of magnesium. The magnesium used in preparing the new alloy and for the purposes of comparison was obtained by subliming commercial magnesium.

Table

| Nominal composition in percent (magnesium—remainder) Ge | Annealed                       |                                  | Cold rolled                    |                                  |
|---------------------------------------------------------|--------------------------------|----------------------------------|--------------------------------|----------------------------------|
|                                                         | Yield strength in lbs./sq. in. | Tensile strength in lbs./sq. in. | Yield strength in lbs./sq. in. | Tensile strength in lbs./sq. in. |
| 0.1                                                     | 7,000                          | 25,000                           | 14,000                         | 24,000                           |
| 0.2                                                     | 9,000                          | 27,000                           | 14,000                         | 27,000                           |
| 0.4                                                     | 11,000                         | 27,000                           | 15,000                         | 27,000                           |
| 0.8                                                     | 11,000                         | 28,000                           | 16,000                         | 27,000                           |
| 4.3                                                     | 15,000                         | 25,000                           | -----                          | -----                            |

The properties set forth above under the term "annealed" were obtained by first rolling the specimens at 550° F. and thereafter annealing them at various temperatures through a range of from 400° to 800° F. The properties selected for the table were those of the annealed specimens which exhibited the maximum elongation. The properties set forth under the term "cold rolled" were obtained by subjecting specimens which had first been hot rolled at a temperature of 550° F. to additional rolling in the cold state. The properties selected for the table were those of the cold rolled specimens which showed the greatest yield and tensile strength, while having at least a 1 per cent elongation in 2 inches.

A comparison of the properties listed in the above table shows the improvement in yield and tensile strengths of my new binary alloy over similar properties of pure magnesium. For example, it will be noted that in the annealed state the yield strength of the new alloy is always superior to that of sublimed magnesium while nearly comparable improvement in the tensile strength prevails in both the annealed and cold rolled state. In addition, it will be noted that the yield strength in the cold rolled state shows improvement in most of the range of the added alloying constituent. The improvement shown in the above compositions is representative of the improvement shown throughout the range of the alloying ingredient indicated.

The new alloy will be found most useful in the production of castings, extruded forms, and the like, wherein high tensile and yield strengths are highly desirable.

The new alloy may be compounded by any of the methods usually employed for melting and alloying metals with magnesium, such as by adding the germanium to a bath of molten magnesium which is preferably protected from oxidation by suitable flux.

I claim:

1. A magnesium base alloy containing from 0.1 to 10 per cent of germanium, the balance being magnesium.
2. A magnesium base alloy containing from 0.5 to 5 per cent of germanium, the balance being magnesium.
3. A magnesium base alloy containing from 0.1 to 10 per cent of germanium and characterized by substantial improvement in at least one of the properties ductility, tensile strength, and yield strength as compared with magnesium without the germanium.

JOHN C. McDONALD.